

L. JONES.

PROCESS OF PRODUCING IRON AND STEEL BARS.

APPLICATION FILED MAR. 1, 1919.

1,354,492.

Patented Oct. 5, 1920.



WITNESSES

*H. M. Irwin Jr.*

INVENTOR

*Llewellyn Jones.*  
BY *Alma Lee*

ATTORNEYS

# UNITED STATES PATENT OFFICE.

LLEWELLYN JONES, OF MUNCIE, INDIANA, ASSIGNOR OF ONE-THIRD TO CHARLES WESTLAKE, JR., OF YOUNGSTOWN, OHIO.

## PROCESS OF PRODUCING IRON AND STEEL BARS.

1,354,492.

Specification of Letters Patent.

Patented Oct. 5, 1920.

Application filed March 1, 1919. Serial No. 280,115.

To all whom it may concern:

Be it known that I, LLEWELLYN JONES, a citizen of the United States, and a resident of Muncie, in the county of Delaware and State of Indiana, have invented certain new and useful Improvements in Processes of Producing Iron and Steel Bars, of which the following is a specification.

My invention relates to improvements in processes of producing bar iron and steel, and it consists in the various steps herein-after described and claimed.

An object of my invention is to provide a process by means of which bar iron and steel may be produced from machine shop turnings more economically than by any other process with which I am familiar.

A further object of my invention is to provide a process by means of which a more homogeneous product is effected and one in which the chemical composition is substantially uniform throughout.

A further object of my invention is to provide a process by means of which bars of better quality, *i. e.*, greater tensile strength, may be produced than by the ordinary process of treating turnings such as that described above.

Other objects and advantages will appear in the following specification and the novel features of the invention will be particularly pointed out in the appended claims.

In the accompanying drawing illustrating my invention,

Figure 1 is a view partly in section and partly in elevation illustrating the first step of compressing the turnings,

Fig. 2 is a perspective view of the receptacle for the turnings, its clamp, and a compacted slug in detached relation,

Fig. 3 is a side view showing the next step with the slug or billet between slabs, with a flux, and

Fig. 4 is a side view of a bar into which the slug is formed after heating.

In carrying out my invention I make use of so called "machine shop turnings" of high and low carbon steel, and wrought iron turnings, also "axle turnings." Turnings at 0.50% to 0.70% carbon may be too high in carbon for use in my process, so I mix with such turnings low carbon turnings, say 0.80% carbon which will give a better fusion. When wrought iron turnings are used the

proper amount of silicon must be introduced 55 to make the metal fuse and weld properly in the subsequent steps of the process. It is of course necessary to vary the proportions of the different grades of turnings to form the particular kind of bar iron or steel 60 desired, that is to say, for a product of a certain composition the mixture would be different from that of a product having another composition.

It will be noted that the mixture is made 65 while the metals are in a cold state. The turnings thus mixed are fed into a suitable press such as a hydraulic press generally indicated at 10 in Fig. 1 wherein the turnings are indicated at 11 in a mold box 12 having 70 a clamping ring 13 and are compressed under high pressure such as exerted by a hydraulic press into slugs or billets 14, the nature of which is such that no apparent or visible interstices remain. A bale or billet 75 is placed on an iron or steel slab or bar 15, and the top of the bale is treated with a flux 16 such as granite dust, borax, lime, aluminum, etc., and a second bar or slab 17 is placed thereon, the layer of flux being 80 between the bale and the upper bar or slab as seen in Fig. 3. The billets are now put into a heating furnace of any suitable type and are heated to approximately 2200° F. or to a suitable welding heat. During this time the 85 flux thoroughly permeates the bales or billets and the impurities are thereby removed from the metal as dross.

The heat treatment brings the metal to the welding point as stated and while it is 90 still hot, it is drawn and rolled into bars such as for instance seen at 18 in Fig. 4. It will be seen that by this process, I avoid the necessity of melting the turnings and subsequently mixing the melted metal with 95 other metal, casting into billets, rolling etc. as has been heretofore necessary. The main features of the present process as distinguished from the ordinary processes are the compressing of turnings which are already 100 mixed and the heating of these compressed bales or billets with a flux which is capable of removing impurities by a heat which brings the metal into condition to be welded and to be rolled into a solid bar.

105 Bars thus produced are homogeneous in texture because of the prior admixture of the proper proportions of metals, and they

are also uniform in chemical composition, while as stated above the process is cheaply carried out.

I claim:

- 5 1. The herein described process of producing commercial iron and steel bars, which consists in mixing scrap metal of high and low carbon content, compressing the cold scrap under sufficiently high pressure to form slugs or billets without apparent or visible interstices, heating the slugs or billets to substantially the welding temperature, and then rolling the heated billets into bars.
- 10 15. 2. The herein described process of producing bar iron or steel from metal turnings which consists in mixing turnings of different chemical composition, compressing the turnings into billets, treating the billets with a flux, heating the billets to substantially the welding temperature whereby the impurities are removed by the flux and rolling the heated billets to form bars.
- 20 3. The herein described process of pro-

ducing bar iron or steel from metal turnings which consists in mixing turnings of different chemical composition, compressing the turnings into porous bales or billets, treating the top of the billets with a flux superposing a bar or slab on each billet, heating the billets and their superposed bars or slabs in a furnace to substantially the welding temperature, and then rolling the billets to form solid bars.

4. The herein described process of producing bar iron or steel from metal turnings which consists in mixing turnings of different chemical composition, compressing the turnings into billets, treating the top of the billets with a flux, superposing a bar or slab on each billet, heating the billets and their superposed bars or slabs to substantially  $2200^{\circ}$  F. whereby the impurities are removed and the metal is brought to a welding temperature and rolling the billets to form solid bars.

LLEWELLYN JONES.